

## UNITED STATES PATENT OFFICE

2,008,602

## PROCESS OF DYEING LEATHER

Fritz Straub and Hans Mayer, Basel, Switzerland, assignors to Society of Chemical Industry in Basle, Basel, Switzerland

No Drawing. Application April 20, 1934, Serial No. 721,640. In Switzerland April 22, 1933

12 Claims. (Cl. 8—5)

This invention relates to a process of dyeing leather fast shades by means of complex metallic compounds of mono-azo-dyestuffs which have the general formula:



10 wherein  $\text{R}_1$  and  $\text{R}_2$  represent aryl residues and  $\text{x}$  a lake-forming group in ortho-position to the azo-group.

15 Complex metallic compounds of mono-azo-dyestuffs of this general formula are, for example, aluminium-, titanium-, vanadium-, chromium-, copper-, manganese-, iron-, cobalt-, nickel- and uranium-compounds of azo-dyestuffs which are obtainable by coupling the diazotized ortho-hydroxy- or ortho-alkoxy- or ortho-carboxy-amino-15  
benzenes or ortho-hydroxy- or ortho-alkoxy- or ortho-carboxyaminonaphthalenes or a derivative  
20 of one of these, for example, a chlorine-, bromine-, nitro-, sulfo-, carboxy-, methoxy- or ethoxy-substitution product with a dihydroxybenzene or a dihydroxynaphthalene for example  
1:3-dihydroxybenzene, 1:3-dihydroxybenzene-4-  
25 carboxylic acid, 1:3-dihydroxybenzene-5-carboxylic acid, 1:2:3-trihydroxybenzene-5-carboxylic acid, 1:5-dihydroxynaphthalene, 2:6-dihydroxynaphthalene or 2:7-dihydroxynaphthalene as well as the sulfonic acids and nitro-, alkyl- or halogen-substitution products of any  
30 of these. These complex metallic compounds may contain one or more metals.

35 The complex metallic compounds to be used dye leather, tanned in any manner, for example, vegetable-tanned leather or chrome-leather, very various tints which are very level and excellently fast.

40 The following examples illustrate the invention:—

Example 1

45 100 parts of neutralized chrome-leather (box calf, chrome sides, goat, kid and sheep) are tumbled in a drum in a bath of 3-400 parts of water at 60° C. During the rotation of the drum,

there is run in, through the hollow axle, a solution (1 part of dyestuff in 50 parts of boiled water) of the nickeliferous dyestuff from the azo-dyestuff of the formula



10 obtainable by coupling diazotized 4-nitro-2-amino-1-hydroxybenzene-6-sulfonic acid with 1:3-dihydroxybenzene. After about 40 minutes the dyestuff has been adsorbed by the leather which is then fatliquored as usual.

15 The leather thus dyed has a brown shade which is very fast.

The leather is dyed through.

Example 2

20 Well tumbled vegetable-tanned sheep or goat leather is dyed, as described in Example 1, with the iron compound of the azo-dyestuff of the formula



30 obtainable by coupling diazotized 4-chloro-2-amino-1-hydroxybenzene with 1:3-dihydroxybenzene. When the dyeing is completed there is added 35 formic acid amounting to half the weight of the dyestuff used and dyeing is continued for 10-15 minutes; the leather is then rinsed.

35 The leather thus dyed has a level full brown-olive shade which is very fast to light.

40 The dyeing can also be conducted by the brushing process with a neutral, cold liquor.

45 The following table gives a series of the dyestuffs serving for the present process and the colours obtained therewith:—

|    | Diazo-component                                        | Coupling component        | Metal                        | Colours obtained |    |
|----|--------------------------------------------------------|---------------------------|------------------------------|------------------|----|
| 50 | (1) 4-nitro-2-amino-1-hydroxybenzene-6-sulfonic acid.  | 1:3-dihydroxybenzene..... | Uranium.....                 | Yellowish brown. | 50 |
|    | (2) 4-nitro-2-amino-1-hydroxybenzene.....              | do.....                   | Manganese.....               | Brown-orange.    |    |
|    | (3) do.....                                            | do.....                   | 80% chromium and 20% nickel. | Janus red.       |    |
|    | (4) do.....                                            | do.....                   | Iron.....                    | Yellow-brown.    |    |
|    | (5) do.....                                            | do.....                   | Cobalt.....                  | Brown-red.       |    |
|    | (6) do.....                                            | do.....                   | Nickel.....                  | Orange.          |    |
|    | (7) 4-chloro-2-amino-1-hydroxybenzene.....             | do.....                   | do.....                      | Do.              | 55 |
|    | (8) do.....                                            | do.....                   | Cobalt.....                  | Bordeaux.        |    |
|    | (9) 5-nitro-2-amino-1-hydroxybenzene.....              | do.....                   | Iron.....                    | Blackish-brown.  |    |
|    | (10) do.....                                           | do.....                   | Cobalt.....                  | Bordeaux.        |    |
|    | (11) do.....                                           | do.....                   | Nickel.....                  | Pink.            |    |
|    | (12) do.....                                           | do.....                   | Manganese.....               | Brown-orange.    |    |
| 60 | (13) 6-nitro-2-amino-1-hydroxybenzene-4-sulfonic acid. | do.....                   | Cobalt.....                  | Brown-violet.    |    |

|    | Diazo-component                                         | Coupling component                      | Metal                                     | Colours obtained    |
|----|---------------------------------------------------------|-----------------------------------------|-------------------------------------------|---------------------|
| 5  | (14) 6-nitro-2-amino-1-hydroxybenzene-4-sulfonic acid.  | 1:3-dihydroxybenzene                    | Nickel                                    | Wine-red.           |
|    | (15) do                                                 | do                                      | Bronze                                    | Blackish-brown.     |
|    | (16) do                                                 | do                                      | Manganese                                 | Violet.             |
|    | (17) 4-nitro-2-amino-1-hydroxybenzene-6-sulfonic acid.  | do                                      | Iron                                      | Brown.              |
| 10 | (18) do                                                 | do                                      | Manganese                                 | Red-brown.          |
|    | (19) do                                                 | do                                      | Cobalt                                    | Do.                 |
|    | (20) 2-amino-1-hydroxybenzene-4-sulfonic acid.          | do                                      | Iron                                      | Brown-orange.       |
|    | (21) do                                                 | do                                      | Manganese                                 | Orange-brown.       |
|    | (22) do                                                 | do                                      | Cobalt                                    | Brown-red.          |
|    | (23) do                                                 | do                                      | Nickel                                    | Brown-orange.       |
|    | (24) do                                                 | do                                      | Chromium and cobalt                       | Bordeaux.           |
|    | (25) 4-methyl-2-amino-1-hydroxybenzene-6-sulfonic acid. | do                                      | Cobalt                                    | Brown-violet.       |
| 15 | (26) do                                                 | do                                      | Uranium                                   | Brown.              |
|    | (27) do                                                 | do                                      | Nickel                                    | Yellow-brown.       |
|    | (28) do                                                 | do                                      | Iron                                      | Olive-brown.        |
|    | (29) do                                                 | do                                      | Manganese                                 | Yellow-brown.       |
|    | (30) 4-chloro-2-amino-1-hydroxybenzene-5-sulfonic acid. | do                                      | Cobalt                                    | Brown-violet.       |
| 20 | (31) do                                                 | do                                      | Nickel                                    | Red-brown.          |
|    | (32) do                                                 | do                                      | Iron                                      | Brown-olive.        |
|    | (33) do                                                 | do                                      | Manganese                                 | Red-brown.          |
|    | (34) 4-chloro-2-amino-1-hydroxybenzene-6-sulfonic acid. | do                                      | Cobalt                                    | Bordeaux.           |
|    | (35) do                                                 | do                                      | Nickel                                    | Brown-red.          |
|    | (36) do                                                 | do                                      | Iron                                      | Olive-brown.        |
|    | (37) do                                                 | do                                      | Manganese                                 | Brown.              |
|    | (38) do                                                 | do                                      | Uranium                                   | Red-brown.          |
| 25 | (39) 5-chloro-2-amino-1-hydroxybenzene-3-sulfonic acid. | do                                      | Iron                                      | Yellowish-brown.    |
|    | (40) 4-chloro-2-amino-1-hydroxybenzene                  | do                                      | Chromium                                  | Bordeaux.           |
|    | (41) 5-nitro-2-amino-1-hydroxybenzene                   | do                                      | do                                        | Violet.             |
|    | (42) 6-nitro-2-amino-1-hydroxybenzene-4-sulfonic acid.  | do                                      | do                                        | Brown-red.          |
|    | (43) do                                                 | do                                      | Copper                                    | Violetish-brown.    |
| 30 | (44) 4-nitro-2-amino-1-hydroxybenzene                   | do                                      | 50 percent chromium and 50 percent nickel | Janus red.          |
|    | (45) 4-chloro-2-amino-1-hydroxybenzene-6-sulfonic acid. | do                                      | Chromium and copper                       | Brown-red.          |
|    | (46) 4-nitro-2-amino-1-phenol                           | 1:3-dihydroxybenzene-4-carboxylic acid. | Chromium                                  | Bordeaux-red.       |
|    | (47) do                                                 | do                                      | Cobalt                                    | Bluish-red.         |
| 35 | (48) do                                                 | do                                      | Nickel                                    | Dull red-brown.     |
|    | (49) do                                                 | do                                      | Manganese                                 | Reddish dark-brown. |
|    | (50) do                                                 | do                                      | Iron                                      | Olive-brown.        |
|    | (51) 5-nitro-2-amino-1-phenol                           | 2:6-dihydroxy-naphthalene               | Chromium                                  | Green-grey.         |
|    | (52) do                                                 | do                                      | Nickel                                    | Dull violet.        |
|    | (53) do                                                 | do                                      | Manganese                                 | Dark grey.          |
|    | (54) do                                                 | do                                      | Iron                                      | Beige-grey.         |
|    | (55) do                                                 | do                                      | Cobalt                                    | Grey-green.         |
| 40 | (56) 6-nitro-2-amino-1-phenol-4-sulfonic acid           | 2:7-dihydroxynaphthalene                | do                                        | Reddish-violet.     |
|    | (57) do                                                 | do                                      | Nickel                                    | Red violet.         |
|    | (58) do                                                 | do                                      | Manganese                                 | Violet brown.       |
|    | (59) do                                                 | do                                      | Iron                                      | Brown blue-violet.  |
|    | (60) do                                                 | do                                      | Chromium                                  | Bluish-violet.      |
|    | (61) 1-aminobenzene-2-carboxylic acid                   | 2:4-dihydroxybenzene                    | do                                        | Full orange.        |
|    | (62) do                                                 | do                                      | Cobalt                                    | Dull light brown.   |
|    | (63) do                                                 | do                                      | Manganese                                 | Reddish-yellow.     |
|    | (64) do                                                 | do                                      | Iron                                      | Light brown.        |
|    | (65) do                                                 | do                                      | Nickel                                    | Reddish-yellow.     |
| 45 | (66) 1-amino-2-ethoxybenzene                            | do                                      | Chromium                                  | Flesh-colored red.  |
|    | (67) do                                                 | do                                      | Cobalt                                    | Light brown.        |
|    | (68) do                                                 | do                                      | Nickel                                    | Do.                 |
|    | (69) do                                                 | do                                      | Manganese                                 | Yellow brown.       |
|    | (70) do                                                 | do                                      | Iron                                      | Reddish-yellow.     |

The azo-dyestuffs of the above table have the following formulas:— (9-12)





What we claim is:—

1. Process of dyeing leather, consisting in using the complex metal compounds of such mono-azo-dyestuffs which correspond to the general formula



wherein  $x$  represents a lake-forming group standing in ortho-position to the azo-bridge,  $\text{R}_1$  is a phenyl radical free from a carboxylic acid group in ortho-position to the lake-forming group and  $\text{R}_2$  is a phenyl or naphthyl radical.

2. Process of dyeing leather, consisting in using the complex metal compounds of such mono-azo-dyestuffs which correspond to the general formula



wherein  $x$  represents a lake-forming group standing in ortho-position to the azo-bridge,  $\text{R}_1$  is a phenyl radical free from a carboxylic acid group in ortho-position to the lake-forming group, and  $\text{R}_2$  is a phenyl radical.

3. Process of dyeing leather, consisting in using the complex metal compounds of such mono-azo-dyestuffs which correspond to the general formula



wherein  $\text{R}_1$  is a phenyl radical free from a carboxylic acid group in ortho-position to the hydroxyl group,  $\text{R}_2$  is a phenyl radical, and the hydroxyl group of the phenyl radical  $\text{R}_1$  stands in ortho-position to the azo-bridge.

4. Process of dyeing leather, consisting in using

70

75

the complex metal compounds of such monoazo-dyestuffs which correspond to the general formula

5



10 wherein  $R_1$  is a phenyl radical free from a carboxylic acid group in ortho-position to the hydroxyl group, and the hydroxyl group of the phenyl radical  $R_1$  stands in ortho-position to the azo-bridge.

15 5. Process of dyeing leather, consisting in using the complex iron compounds of such monoazo-dyestuffs which correspond to the general formula

20



25 wherein  $R_1$  is a phenyl radical free from a carboxylic acid group in ortho-position to the hydroxyl group, and the hydroxyl group of the phenyl radical  $R_1$  stands in ortho-position to the azo-bridge.

30 6. Process of dyeing leather, consisting in using the complex iron compound of the monoazo-dye-stuff of the formula

35



40 7. As new compositions of matter of yellow, brown, red, violet and green tint, the coloured leather dyed fast with the complex metal compounds of such monoazo-dyestuffs which correspond to the general formula

45



50 wherein  $x$  represents a lake-forming group standing in ortho-position to the azo-bridge,  $R_1$  is a phenyl radical free from a carboxylic acid group in ortho-position to the lake-forming group and  $R_2$  is a phenyl or naphthyl radical.

55 8. As new compositions of matter of yellow-brown, brown, red and violet tint, the coloured leather dyed fast with the complex metal compounds of such monoazo-dyestuffs which correspond to the general formula

60



wherein  $x$  represents a lake-forming group stand-

ing in ortho-position to the azo-bridge,  $R_1$  is a phenyl radical free from a carboxylic acid group in ortho-position to the lake-forming group, and  $R_2$  is a phenyl radical.

9. As new compositions of matter of yellow-brown, brown, red and violet tint, the coloured leather dyed fast with the complex metal compounds of such monoazo-dyestuffs which correspond to the general formula

5



10 wherein  $R_1$  is a phenyl radical free from a carboxylic acid group in ortho-position to the hydroxyl group,  $R_2$  is a phenyl radical, and the hydroxyl group of the phenyl radical  $R_1$  stands in ortho-position to the azo-bridge.

15 10. As new compositions of matter of yellow-brown, brown, red and violet tint, the coloured leather dyed fast with the complex metal compounds of such monoazo-dyestuffs which correspond to the general formula

20



25 wherein  $R_1$  is a phenyl radical free from a carboxylic acid group in ortho-position to the hydroxyl group, and the hydroxyl group of the phenyl radical  $R_1$  stands in ortho-position to the azo-bridge.

30 11. As new compositions of matter of brown tint, the coloured leather dyed fast with the complex iron compound of such monoazo-dyestuffs which correspond to the general formula

35



35 wherein  $R_1$  is a phenyl radical free from a carboxylic acid group in ortho-position to the hydroxyl group, and the hydroxyl group of the phenyl radical  $R_1$  stands in ortho-position to the azo-bridge.

40 12. As new composition of matter of brown tint, the coloured leather dyed fast with the complex iron compound of the monoazo-dye-stuff of the formula

45



FRITZ STRAUB.  
HANS MAYER.